

J. W. NYSTROM.  
Making Bessemer Steel.

No. 33,446.

Patented Oct. 8, 1861.



Witnesses:

Wm H. Harrison

A. C. Tommons

John W. Nystrom by  
A. A. Leeks, Secy.

# UNITED STATES PATENT OFFICE.

JOHN W. NYSTROM, OF PHILADELPHIA, PENNSYLVANIA.

## IMPROVEMENT IN FURNACES FOR THE MANUFACTURE OF IRON AND STEEL.

Specification forming part of Letters Patent No. 33,446, dated October 8, 1861.

*To all whom it may concern:*

Be it known that I, JOHN W. NYSTROM, of the city and county of Philadelphia, in the State of Pennsylvania, have invented certain new and useful improvements in the construction, arrangement, and operation of furnaces destined for the manufacture of iron and steel; and I hereby declare that the following, taken in connection with the accompanying drawings, is a full, clear, and exact description of the same.

My invention consists, first, in the construction of a barrel-furnace in which one or more tuyeres are arranged at such an angle in relation to the curved bottom of the furnace that the blast shall be tangent, or nearly so, to the said bottom, and agitate the molten mass by passing along the interior or concave surface of the furnace, substantially in the manner and for the purposes hereinafter described; second, in the combination, with a barrel-furnace constructed and arranged essentially as described, of a front plate capable of removal, substantially as and for the purpose hereinafter set forth; third, in providing a barrel-furnace arranged and operated as hereinafter described with a friction-strap or its mechanical equivalent, to firmly hold and prevent shaking of the furnace during the operation of decarbonization, substantially as herein-after specified; fourth, in the formation of a flue or chimney uniting the barrel-furnace with the cupola or blast furnace, essentially as hereinafter shown and described, so that particles of iron carried off with the air or gases or other volatile products may be returned to the furnace, and thus be utilized again; fifth, in so forming and arranging the outlet of a barrel-furnace constructed and operated as hereinafter described as that it shall occupy, when the furnace is in position to be emptied, the lowest part of the concave bottom.

To enable others skilled in the art to make and use my improvements, I shall now proceed to describe the construction, arrangement, and operation of the furnace, referring to the accompanying drawings, in which—

Figure 1 represents a cross-section of my improved furnace as combined with an ordinary cupola; Fig. 2, a longitudinal section of the same through the line A B in Fig. 1, and

Fig. 3 a plan view of an arrangement of several furnaces with their cupolas.

The furnace F, it will be seen, is formed into the shape of a barrel placed horizontally and supported at one end by a hollow trunnion, G, resting in suitable bearings, while at the other end it is held in position by means of two friction-rollers, f f. The front or cap, E, the inside of which is lined with fire clay and brick, is screwed or clamped or otherwise securely attached to the end of the furnace, so that it may be easily removed when the inside of the furnace is to be built up, repaired, or cleaned out.

In the drawings, H represents the mass of molten cast-iron to be decarbonized on the well-known principle by blowing air into or through it. The air is conveyed from a suitable blowing engine through the pipe and passages a a, and is blown into the furnace through the tuyeres b b, which are placed in an inclined position of about forty-five degrees, tangenting the curved bottom of the furnace. By thus arranging the tuyeres a more thorough and regular circulation is imparted to the mass of molten iron. The carbonic-acid gas formed in the furnace is conveyed off by the chimney C into the cupola or blast furnace P. Particles of iron that are carried off with the air, gases, or other volatile products engendered during the carbonization of the iron will be thus collected and utilized in the cupola or blast furnace, while additional heat for the melting of the cast-iron or the smelting of the ore will be attained. The frame h contains the friction-rollers f f and strap i, which are arranged in the front end of the furnace, the former to support that end of the furnace, and the latter, by being stretched by the lever and screw k k around the front end of the furnace against the friction-rollers f f, to keep it steady during the operation of blowing air into the molten metal. Other means may be resorted to, however, to prevent the violent shakings of the furnace, such as clamps, weights, wedges, screws, &c.; but I have described a simple and efficient device to effect the purpose. The outer shell of the furnace I prefer to make of wrought-iron, riveted to the back I.

In the shell of the furnace opposite the tuyeres are inserted removable glasses n n for the purpose of looking through into the fur-

nace during the operation, and also for cleaning the tuyeres. The furnace is moved around its axis by means of lever *l*, fastened to the back *I*, as shown in the plan view, Fig. 3. By this lever the furnace is placed in the different positions required during the operation.

When the furnace is to be filled with molten iron, it is turned so that the mouth *c* comes to *c'* under the spout *S*. The iron may be thus run directly from the cupola or blast furnace into the furnace *F*.

In order to clean the furnace out from slag, &c., it is turned so that the mouth *c'* comes down toward the corner *o*, when part of the slag will run out, the remainder being removed by suitable tools or implements. The furnace may be turned by gearing, worm-screw, or other mechanism. It is intended here to turn the furnace by means of ropes and pulleys, the former fastened to the end of the lever *i*, while the latter is secured to some convenient place in or near the ceiling or roof of the foundry. When the iron is decarbonized, the furnace is turned so that the opening *d* comes to *d'*, in which position it is allowed to remain for a few minutes, so that the slag and other light impurities may rise to the surface of the molten mass. The fluid metal is then let out through the aperture *d*, either directly into a mold or chill, *D*, or by the spout *s* to the mold *L*. The outlet *d'*, being at the bottom of the vessel, lets out the pure iron or steel first, while the slag and lighter impurities remain on the surface of the molten mass, thus producing a good, pure casting.

Fig. 3 shows how to arrange several furnaces, *F*, and cupolas *P*, for the purpose of casting large and long pieces. Any number of furnaces and cupolas may be employed in this way. On one side of the cupolas the blast is led through a pipe or column, *m*, into the furnaces *F*, and by the pipes *g* into the cupolas. The pit for casting large and long pieces branches off under the furnaces, as shown in the drawings. Boards *ee* are placed for crossing the pit. This seems to be a good arrangement; but it can also be arranged with a long pit directly under the furnaces, as shown on the other side of the cupolas.

The operation is conducted in the following manner: The cast-iron is first melted down in the cupola *P*. The furnace *F* is turned by the lever *l*, so that the mouth *c* comes to *c'* under the spout *S*. When the cast-iron is melted, it is let out in the ordinary way and conducted by the spout *S* directly into the furnace *F*, until it is about half-full, which will be indicated by the fluid mass being in the barrel-furnace on a level with the mouth *c'*. The spout *S* is then drawn aside, the blast

turned on, and the furnace moved by the lever *l* until the mouth *c* butts up close to the chimney *C*. The furnace is now clamped fast to the friction-rollers, and the operation of decarbonizing the iron is continued for from five to fifteen minutes, according to the kind of iron or steel that it is intended to be obtained. The strap *i* is now loosened by the screw and lever *k*, the furnace turned to its former position, when the outlet *d* will come to *d'*, through which the fluid iron or steel is either cast directly into a mold or chill, *D*, or is conducted by means of spout *s* into the mold *L*. The casting may then be taken directly to a steam-hammer or rolling-mill and forged in the same heat.

For very large castings it will be necessary to employ several furnaces, as shown in Fig. 3, when the same operation must go on simultaneously in all of them.

Having thus fully described my invention, what I claim, and desire to secure by Letters Patent, is—

1. The construction and arrangement of furnaces capable of rotation upon a horizontal axis, and having tuyeres so arranged in an inclined position that the blast enters the molten iron tangentially, or nearly so, to the curved bottom of such furnaces.

2. The combination, with a barrel-furnace constructed and arranged essentially as described, of a front plate capable of removal, substantially as and for the purpose herein set forth.

3. Providing a barrel-furnace arranged and operated as herein described with a friction-strap or its mechanical equivalent to firmly hold and prevent shaking of the furnace during the operation of decarbonization, substantially as herein set forth.

4. In combination with a furnace capable of rotation, as described, and provided with a mouth for the reception of the molten metal from the cupola, the side chimney on the cupola so arranged that the said mouth shall come in juxtaposition with and convey the gases to the chimney, as described.

5. So forming and arranging the outlet of a barrel-furnace constructed and operated as herein described as that it shall occupy, when the furnace is in position to be emptied, the lowest part of the concave bottom.

In testimony whereof I have signed my name to this specification before two subscribing witnesses.

Washington, September 7, 1861.

JOHN W. NYSTROM,

Witnesses:

A. POLLAK,

EDM. F. BROWN.